

[54] **PROCESS FOR THE SINGLE-BATH DYEING OF CELLULOSE AND POLYAMIDE FIBER BLENDS ACCORDING TO THE PAD DYEING TECHNIQUE**

[75] Inventors: **Hans-Ulrich von der Eltz, Frankfurt/Main; Hans-Peter Maier, Sulzbach/Taunus; Dietfried Suchy, Fulda, all of Germany**

[73] Assignee: **Farbwerke Hoechst Aktiengesellschaft Vormals Meister Lucius & Bruning, Frankfurt/Main, Germany**

[22] Filed: **Feb. 23, 1972**

[21] Appl. No.: **228,756**

[30] **Foreign Application Priority Data**

Feb. 25, 1971 Germany ..... 2108875

[52] U.S. Cl. ..... 8/21 B, 8/26

[51] Int. Cl. ..... D06p 3/82

[58] Field of Search ..... 8/21 B, 25, 21 A, 163, 26

[56] **References Cited**

UNITED STATES PATENTS

3,097,040 7/1963 Casty ..... 8/163 X

3,252,963 5/1966 Blackhall et al. ..... 260/147  
3,293,238 12/1966 Chang ..... 260/153

FOREIGN PATENTS OR APPLICATIONS

1,155,148 6/1969 Great Britain ..... 8/21 B  
652,584 8/1964 Belgium ..... 8/21 B

Primary Examiner—Herbert B. Guynn

Assistant Examiner—Bruce H. Hess

Attorney, Agent, or Firm—Curtis, Morris & Safford

[57] **ABSTRACT**

Process for the single-bath dyeing of blends of cellulose fibers and synthetic polyamide fibers with reactive dyestuffs and non-reactive metal complex dyestuffs according to a continuous or semi-continuous method of the pad dyeing technique, by applying to these fibrous materials aqueous padding liquors which contain alkaline agents in addition to combinations of the above-mentioned dyestuffs, and then, optionally after intermediate drying, submitting the material so treated in the alkaline medium to the action of heat or allowing it to dwell at room temperature or at slightly elevated temperature for the fixation of the dyestuffs.

8 Claims, No Drawings

PROCESS FOR THE SINGLE-BATH DYEING OF  
CELLULOSE AND POLYAMIDE FIBER BLENDS  
ACCORDING TO THE PAD DYEING TECHNIQUE

The present invention relates to a process for the single-bath dyeing of cellulose and polyamide fiber blends according to a continuous or semi-continuous method of the pad-dyeing technique.

It is known that textile materials of cellulose fibers can be dyed with reactive dyestuffs by reacting them with the hydroxyl groups of the cellulose fibers under alkaline conditions. Pad-dyeing methods are of particular importance in this field because they can be carried out in fully or semi-continuous manner. For the fixation of the above dyestuffs on cellulose fabrics, an important and economic dyeing technique is represented by the pad-batch process at which dyestuff and alkali are applied together to the fiber and fixation of the wound-up dyeing ensues at room temperature within a certain dwelling time [cf. SVF-Fachorgan 16, (1961), pages 320-340]. In the dyeing of blended fabrics of cellulose and polyamide fibers this application method could only be employed, up to now, for the cellulose fiber portion of the textile material, in which case dyeing of the polyamide fiber component had to be effected by cross-dyeing, subsequent to the after-treatment of the reactive dyeing, in discontinuous manner with acid, metal complex or disperse dyestuffs from an acid or neutral medium at the boiling temperature or at an elevated temperature. This two-bath dyeing method has the drawback that it is very complicated and allows no continuous working. The same applies when working according to the pad drying process.

However, blended fabrics of native or regenerated cellulose fibers and synthetic polyamide fibers can be dyed or printed continuously according to the thermosol process with disperse and reactive dyestuffs. According to this single-bath dyeing technique an aqueous composition which contains in addition to disperse and reactive dyestuffs also alkali as well as, optionally, further additives such as cross-linking and thickening agents, is applied to the textile material, then the fabric is dried and submitted to a heat treatment at about 175° - 220°C for 30 to 60 seconds. By the thermosol operation, the polyamide fiber portion of the blended fabric is fixed and is, thus, imparted its optimum technological properties. At the same time, the disperse dyestuff is fixed on the polyamide fiber and the reactive dyestuff on the cellulose fiber. This process, however, is very expensive because of the dyestuffs used; the fastness properties, especially those as to wet processing of the dyeings are not satisfactory in many cases.

Now, it has been found that the above-cited difficulties and drawbacks can be overcome and that blends of cellulose fibers and synthetic polyamide fibers can be dyed with reactive dyestuffs and non-reactive metal complex dyestuffs according to a fully or semi-continuous single-bath method of the pad-dyeing technique when applying to these fibrous materials aqueous padding liquors which contain alkaline agents besides combinations of the above-mentioned dyestuffs, and then optionally after intermediate drying, exposing the material thus treated in the alkaline medium to the action of heat or allowing it to dwell at room temperature or at slightly elevated temperature for the fixation of the dyestuffs.

This process allows combinations of one or several reactive dyestuffs and of one or several metal complex dyestuffs to be simultaneously fixed on the fiber blends, the reactive dyestuff substantially dyeing the cellulose fiber portion of the material and the metal complex dyestuff and, as the case may be, further proportions of the reactive dyestuff, dyeing the polyamide component. This result could not be foreseen by those skilled in the art and it is, thus, extraordinarily surprising that metal complex dyestuffs can be fixed on the polyamide material in water-soluble or dispersed form by a heat-treatment, especially under alkaline conditions. Such a result was the more surprising as the specialist knows that the disperse or acid dyestuffs usually employed for dyeing polyamide fibers are more or less destroyed at the elevated temperatures of the thermosol process under alkaline conditions and that reproducible and level dyeings cannot be obtained for this reason. According to the invention it could not be expected that metal complex dyestuffs may be fixed on polyamides — especially from an alkaline medium — by dwelling at room temperature since the pad dwell process generally does not allow to obtain reproducible and level dyeings with the dyestuffs otherwise suitable for polyamide fibers, especially with acid and disperse dyestuffs, at room temperature.

According to this invention the textile material is impregnated on a padding machine at 20°C to 25°C with an aqueous padding liquor containing the dissolved reactive dyestuff, the dissolved or dispersed metal complex dyestuff, alkaline substances and, optionally, further auxiliary additives, and then freed from the excess liquid.

For the fixation of the dyestuff mixtures applied in this manner by which the fixing operation is carried out under the action of heat, there are available different methods:

Thus, for example, the fibrous material can be submitted in moist state, immediately after having been padded with the dyestuff preparation, to a steam process of from 30 to 180 seconds, preferably from 30 to 60 seconds, at a temperature within the range of from 100° to 108°C, preferably of from 103° to 105°C. (one-bath pad wet-steam process). Along another procedure, the pad-dyeings can also be steamed, after an intermediate drying step at relatively low temperatures up to 110°C, for 5 to 15 minutes, preferably for 7 to 10 minutes, at a temperature from 100° to 108°C, preferably at from 100° to 105°C (one-bath pad-steam process), or they can be thermosoled on a tenter frame or a sieve drum drier by forcing through the goods dry hot air by suction or by contact heating at temperatures within the range of from 190° to 220°C within from 10 to 60 seconds, preferably for 60 seconds at 195°C (heat fixation process). Intermediate drying after the padding process may, however, be omitted if, by treating the padded material, for example, on the hot-flue, for 1 to 6 minutes, preferably for 90 to 120 seconds, at temperatures within the range of from 130° - 170°C, preferably at about 140°C, together with the drying of the goods, fixation of the dyestuff is effected (one-bath pad drying process). The various possibilities of a heat fixation described above according to the present invention offer, simultaneously with the single bath processing, above all the special advantage of a continuous operation technique. The large tolerance with regard to the fixation temperature and/or fixation time is bal-

anced according to the claimed process by variation of the alkali concentration. By means of these operating methods very high speeds of the goods can be obtained. Furthermore, the results of the dyeing can be reproduced to a high degree.

The favourable conditions offered by the single-bath dyeing method are maintained when the blended fabrics padded simultaneously with the dyestuff combinations and with alkali are rolled onto a beam and the fibrous material is allowed to dwell in moist state at room temperature or at slightly elevated temperature within the range of from 30° to 60°C for 2 to 24 hours, preferably for 8 to 14 hours (one-bath pad-batch process or short-time pad-batch process). This semi-continuous dyeing technique is characterized by a high degree of utility because of the energy saved and expensive aggregates for intermediate drying and fixing are not necessary.

After dyeing, the material is rinsed, soaped and finished in usual manner. When pursuing the working conditions described above, the metal complex dyestuff causes no or only little soiling of the cellulose portion. For the dyeing with the reactive dyestuffs it is important that during the washing process the aqueous baths are not neutralized with acetic acid, since otherwise part of the reactive dyestuff is fixed on the polyamide fiber portion of the material which causes a change in shade.

The process of the invention for dyeing textile materials which consist of cellulose and polyamide fiber blends has the advantage, in comparison with the single-bath dyeing technique generally used for this purpose, that considerably improved fastness properties can be obtained, especially with respect to wet processing. For example, the fastness to perspiration of the dyeings was given the mark 5, a result which could not be obtained by other methods, especially by the single-bath dyeing technique mentioned as prior art. The two-bath processes for dyeing the said fiber blends are surpassed by the novel process in that the working methods are simplified and the costs are reduced.

In the process of the invention, preferably such reactive dyestuffs are used which contain, as the reactive component, at least one vinylsulfone group or at least one group capable of forming the vinylsulfone group under the action of the alkaline agents during the dyeing process. In this case, it is not important whether the said radicals are bound to the dyestuff molecule directly or via a bridge member, especially —NH— or —NR— (R = lower alkyl). Among the groupings which can be converted into the reactive vinylsulfone group by alkaline substances, there may be mentioned, for example, the  $\beta$ -sulfatoethyl-sulfone group, the  $\beta$ -thiosulfatoethyl-sulfone group, the  $\beta$ -phosphatoethyl-sulfone group, the  $\beta$ -chloroethyl-sulfone group, the  $\beta$ -dialkylaminoethyl-sulfone group as well as the corresponding sulfonylamino groups, especially the ethylenylamino radical. All the other known reactive dyestuffs, especially those which contain, as the reactive group, at least one  $\beta$ -(2,2,3,3-tetrafluorocyclobutyl)-acrylamino- or  $\beta$ -(2,2,3,3-tetrafluoro-4-alkylcyclobutyl)-acrylamino group can be used for the novel dyeing method. As parent substances for these dyestuffs there are especially suitable those of the anthraquinone, azo and phthalocyanine dyestuff series, in which case the azo and phthalocyanine dyestuffs may

be metal-free or metallized.

As non-reactive metal complex dyestuffs there are used in the process of this invention 1:2-chromium or cobalt complex compound of azo dyestuffs, especially 5 monoazo dyestuffs, i.e. compounds in which 2 molecules of one azo dyestuff or 1 molecule each of two azo dyestuffs different from one another are bound to a chromium or cobalt atom in complex-bound form. The complex may contain, for example, one disazo dyestuff 10 and one monoazo dyestuff or, preferably, two identical or different monoazo dyestuff molecules. Furthermore, there may be used water-soluble, metallized azo dyestuffs which contain per dyestuff molecule only one metal atom in complex bound form (1:1-metal complex 15 compounds), especially copper, and also chromium or cobalt. These azo dyestuffs contain as groups forming the metal complex linkage preferably o,o'-dihydroxy azo groupings.

According to the above process, there may be used 20 in the padding liquors, on principle, all inorganic substances having an alkaline effect, such as sodium carbonate, sodium bicarbonate, trisodium phosphate, disodium phosphate, sodium hydroxide, sodium silicates, the corresponding potassium compounds or mixtures 25 of these alkalis in amounts of from 3 to 30 g, preferably from 5 to 20 g, per liter of padding liquor, said alkali content depending, on the one hand, on the dyestuff amounts used and, on the other hand, on the efficiency 30 of the energy supplied for fixation. The pH-value of the dyebath generally is within the range of from 8 to 13.

Depending on the type of the fixation method, the padding liquors may advantageously contain electrolytes, especially crystallized sodium sulfate or purified sodium chloride in amounts ranging from 10 to 40 g, 35 preferably of about 30 g, per liter of padding liquor.

Commercial wetting and thickening agents may also be added to the dyebaths used, a capillary-active mixture containing branched aliphatic carboxylic acid esters, optionally partially saponified phosphoric acid esters of aliphatic alcohols of medium molecular weight, small amounts of fatty acids or soaps and as wetting agent known higher oxalkylates of aliphatic or aliphatic-aromatic sulfonic acids being especially recommended, since it advantageously influences the intensity and levelness of shade. Similar good effects with regard to the colour yield and the levelness are provided by alkali metal salts of the m-nitro-benzenesulfonic acid and the polyalkylene glycols, preferably polyethylene glycols, having an average molecular weight of about 400 to 800. The above-mentioned auxiliaries are used in amounts within the range of from 5 to 20 g/l, preferably 10 to 15 g/l of the dyeing preparation.

55 The textile material to be dyed in accordance with the invention which consists of blends of native or regenerated cellulose fiber and synthetic polyamides in a ratio of from 50 : 50 to 85 : 15 has the working stage of a flat-surface textile structure, for example a woven or knitted fabric.

60 The following Examples serve to illustrate the invention, the parts and percentages being by weight, unless otherwise stated.

#### EXAMPLE 1

65 16 g of the reactive dyestuff of formula



were dissolved in the two to four fold amount of hot water and this solution was cooled to about 50°C by adding about the same amount of cold water. Another aqueous dyestuff solution prepared in the same manner by using 8 g of the 1:2-chromium complex compound of the dyestuff of formula



10 g of m-nitrobenzenesulfonic acid (sodium salt) and 10 g of crystallized sodium sulfate, was poured into the solution of the reactive dyestuff and the mixture was made up to a volume of 1 liter by adding cold water.

Furthermore, 15 g of sodium bicarbonate were added to the dye bath thus prepared.

- With this padding liquor, a blended fabric of cotton and synthetic polyamide fibers in the ratio of 60 : 40 was impregnated at 20° to 25°C on a padding machine and freed from the excess liquid by squeezing, then it was submitted to intermediate drying at 90° to 100°C on a hot-flue and subsequently steamed at 100° to 105°C for 7 to 10 minutes. Then, the fabric thus dyed was rinsed with neutral, cold water and then with hot water of about 80°C and soaped at room temperature for 5 minutes with a solution containing 1 g of a condensation product of oleic acid and N-methyl-taurine (as sodium salt) per liter of water.
- 15 After rinsing with hot and cold water and drying had been repeated, a dyeing was obtained in which the cotton fiber portion of the material was dyed in orange shade and the polyamide fiber component in dark blue shade.
- 20 The following Table 1 indicates further dyestuff combinations which may be used for the dyeing of blended fabrics of cellulose and polyamide fibers according to the method described in Example 1, the dyestuff amounts to be used in each case and the shades obtainable on the fiber blend components:

TABLE 1

| Example | Dyestuff combination | Amount, grams | Shade                           |
|---------|----------------------|---------------|---------------------------------|
| 2       |                      | 15            | Cotton fiber: brilliant yellow. |
|         |                      | 19            | Polyamide fiber: navy blue.     |
|         |                      | 1.6           |                                 |
| 3       |                      | 17            | Cotton fiber: intense yellow.   |

TABLE 1—Continued

| Example | Dyestuff combination                                                                                                | Amount, grams | Shade                         |
|---------|---------------------------------------------------------------------------------------------------------------------|---------------|-------------------------------|
|         | <br>1:1-chromium complex compound. | 13            | Polyamide fiber: blue.        |
| 4       | <br>(CuPc=copper phthalocyanine). | 11            | Cotton fiber: turquoise blue. |
|         | <br>1:2-chromium complex compound. | 12            | Polyamide fiber: red.         |

## EXAMPLE 5

16 g of the reactive dyestuff of the formula



30



35 10 g of m-nitrobenzenesulfonic acid (sodium salt) and 30 g of crystallized sodium sulfate, was poured into the solution of the reactive dyestuff and the mixture was made up to a volume of 1 liter by adding cold water. Furthermore, 16 cc. of sodium hydroxide solution of 38°Be were added to the dyebath thus prepared.

40 With this padding liquor, a blended fabric of cotton and synthetic polyamide fibers in the ratio of 60 : 40 was impregnated at 20° to 25°C on a padding machine and freed from the excess liquid by squeezing and then steamed without intermediate drying at 103° to 105°C for 60 seconds. Subsequently, the fabric thus dyed was rinsed in the same way as described in Example 1, after-treated and finished. A dyeing was obtained in which the cotton fiber portion of the material was dyed in golden-yellow shade and the polyamide fiber component in bordo shade.

45 55 Further dyestuff combinations suitable for the dyeing of blended fabrics of cellulose and polyamide fibers as indicated in Example 5, the dyestuff amounts to be used in each case and the shades obtainable on the components of the fiber blend in these cases are indicated in the following Table 2:

TABLE 2

| Example | Dyestuff combination                                                                 | Amount, grams | Shade                 |
|---------|--------------------------------------------------------------------------------------|---------------|-----------------------|
| 6       |  | 17            | Cotton fiber: orange. |

TABLE 2—Continued

| Example | Dyestuff combination | Amount,<br>grams | Shade                       |
|---------|----------------------|------------------|-----------------------------|
| 9       |                      | 9                | Polyamide fiber: dark blue. |
| 7       |                      | 13               | Cotton fiber: turquoise.    |
| 8       |                      | 13               | Polyamide fiber: red.       |
| 8       |                      | 10               | Cotton fiber: yellow.       |
|         |                      | 5                |                             |
|         |                      | 12               | Polyamide fiber: navy blue. |
|         |                      | 8                |                             |
|         |                      |                  |                             |

## EXAMPLE 9

8 g of the reactive dyestuff of the formula



8 g of the 1:2-cobalt compound of the dyestuff of formula

10



and 11 g of the 1:2-chromium complex compound of the dyestuffs of formula



were flooded with about 200 cc. of boiling water and dissolved while stirring thoroughly. After having added 500 cc. of cold water 10 g of m-nitrobenzenesulfonic acid (sodium salt), 10 g of crystallized sodium sulfate and 20 g of calcined sodium carbonate were stirred in this solution whereupon the dyebath so prepared was made up to a volume of 1 liter by adding cold water.

With this padding liquor, a blended fabric of cotton and synthetic polyamide fibers (ratio 50 : 50) was impregnated at 20° to 25°C, freed from the excess liquid by squeezing and then dried at 140°C for 90 to 120 seconds on a hotflue. Subsequently, the material thus treated was rinsed in the way indicated in Example 1, soaped with a non-ionic detergent and finished. A dyeing was obtained in which the cotton component of the fiber blend was dyed in scarlet red shade and the polyamide fiber component in dark blue shade.

## EXAMPLE 10

An aqueous solution was prepared from 35 g of the reactive dyestuff of the formula



and from 16 g of the 1:2-cobalt complex compound of the dyestuff of the formula



15

in the same manner as described in Example 9, the additives indicated therein were added and it was made up to a dyebath volume of 1 liter by adding water.

With the padding liquor so prepared, a cotton/polyamide blended fabric in the ratio of 50 : 50 was dyed in the same manner as described in Example 9, and, upon the aftertreatment, a dyeing was obtained in which the cotton fiber portion of the material was dyed in navy blue shade and the polyamide component in red violet shade.

## EXAMPLE 11

16 g of the reactive dyestuff of the formula



were dissolved in the two to four fold amount of hot water and this solution was cooled to about 50°C by adding cold water. Another aqueous dyestuff solution prepared in the same manner using 10 g of the 1:2-cobalt complex compound of the dyestuff of formula



and 20 g of a polyethylene glycol having an average molecular weight of about 400, was poured into the solution of the reactive dyestuff and the mixture was made up to a bath volume of 1 liter by adding cold water. Furthermore, 10 g of sodium bicarbonate were added to the dyebath so prepared.

With this padding liquor, a blended fabric of equal proportions of cotton and of synthetic polyamide fibers

was impregnated at 20° to 25°C on the padding machine and squeezed, then dried at 110°C and thermosoled at 190°C for 30 to 60 seconds by means of hot air on a tenter frame. Subsequently, the fabric thus dyed was rinsed with neutral, cold water and then with hot water at about 80°C and soaped at room temperature for 5 minutes with a solution containing 1 g of the condensation product of oleic acid and N-methyl tau-

5  
10

rine (as sodium salt) per liter of water. After rinsing and drying had been repeated a dyeing was obtained

in which the cotton fiber portion of the blended fabric was dyed in ruby-red shade and the polyamide fiber component in orange shade.

The following Table 3 indicates further Examples of dyestuff combinations for the dyeing of blended fabrics of cellulose and polyamide fibers according to the method indicated in Example 11, the dyestuff amounts to be used in each case and the shades obtainable on the components of the fiber blend in these cases:

TABLE 3

| Example | Dyestuff combination | Amount, grams | Shade                       |
|---------|----------------------|---------------|-----------------------------|
| 12      |                      | 17            | Cellulose fiber: yellow.    |
| 13      |                      | 16            | Polyamide fiber: red.       |
| 14      |                      | 26            | Cellulose fiber: navy blue. |
| 14      |                      | 12            | Polyamide fiber: brown.     |
| 14      |                      | 15            | Cellulose fiber: blue.      |
| 14      |                      | 13            | Polyamide fiber: bordo.     |

1:2-cobalt complex compound.



TABLE 3—Continued

| Example | Dyestuff combination | Amount, grams | Shade                        |
|---------|----------------------|---------------|------------------------------|
| 15..... |                      | 11            | Cellulose fiber: orange.     |
|         |                      | 4             | Polyamide fiber: anthracite. |
|         |                      | 7             |                              |
|         |                      | 13            |                              |
|         |                      | 1             |                              |
|         |                      | 8             | Cellulose fiber: yellow.     |
| 16..... |                      | 7             |                              |
|         |                      | 4             | Polyamide fiber: anthracite. |
|         |                      | 7             |                              |
|         |                      | 1             |                              |

TABLE 3—Continued

| Example | Dyestuff combination                  | Amount,<br>grams | Shade |
|---------|---------------------------------------|------------------|-------|
|         | <p>1:2-chromium complex compound.</p> | 13               |       |

**EXAMPLE 17**

15 g of the reactive dyestuff of the formula



were dissolved in the two to four fold amount of hot water and this solution was cooled to about 50°C by adding cold water. Another aqueous dyestuff solution prepared in the same manner using 17 g of the 1:2-chromium complex compound of the dyestuffs of formula



15 was poured into the solution of the reactive dyestuff and the mixture was made up to a volume of 1 liter by adding cold water. Furthermore, 5 g of a capillary-active mixture containing esters of branched fatty acids having from six to 12 carbon atoms and of low molecular secondary alkanols, phosphoric acid esters of alkanols having from four to 8 carbon atoms, small amounts 20 of fatty acids having from 12 to 18 carbon atoms or the salts thereof and alkansulfonic acids having from 10 to 20 carbon atoms, 16 cc. of sodium hydroxide solution of 38°Be and 30 g of crystallized sodium sulfate were added to the dyebath so prepared.

25 With this padding liquor, a blended fabric of equal proportions of cotton and of synthetic polyamide fibers was impregnated at 20° to 25°C on a padding machine, squeezed and then rolled up in moist state. To protect the padded material from irregular drying the rolled up  
30 textile material was enveloped in a plastic sheet and was allowed to dwell in this state at room temperature for 12 hours for dyestuff fixation. Then, the fabric thus dyed was first thoroughly rinsed with neutral cold water and then with hot water at 80°C and soaped for 5 minutes at the boiling point with a solution containing per liter of water 1 g of the condensation product of oleic acid and N-methyltaurine (as sodium salt). After rinsing with hot and cold water had been repeated a dyeing was obtained in which the cotton fiber component was  
35 dyed in yellow shade and the polyamide fiber component in blue shade.

The following Table 4 indicates further dyestuff combinations suitable for dyeing cellulose and polyamide fiber blends in a manner described in Example 17, this 45 summary also containing the dyestuff amounts to be used in each case and the shades obtainable on the blended fabric:

TABLE 4

| Example | Dyestuff combination | Amount,<br>grams | Shade                    |
|---------|----------------------|------------------|--------------------------|
| 18.     |                      | 15               | Cellulose fiber: yellow. |
|         |                      | 12               | Polyamide fiber: blue.   |

TABLE 4—Continued

| Example | Dyestuff combination                                                                                                                                                           | Amount,<br>grams | Shade                            |
|---------|--------------------------------------------------------------------------------------------------------------------------------------------------------------------------------|------------------|----------------------------------|
| 19      |  <p>(CuPc=copper phthalocyanine).</p> <p>1:2-chromium complex compound.</p>                   | 13               | Cellulose fiber; turquoise blue. |
|         |                                                                                                                                                                                | 12               | Polyamide fiber; dark orange.    |
| 20      |  <p>(NiPc=nickel phthalocyanine).</p> <p>1:1-chromium complex compound (mixed chroming).</p> | 21               | Cellulose fiber: turquoise blue. |
|         |                                                                                                                                                                                | 15               | Polyamide fiber: black.          |
| 21      |  <p>1:2-cobalt complex compound.</p>                                                        | 16               | Cellulose fiber: bordo.          |
|         |                                                                                                                                                                                | 7                | Polyamide fiber: red violet.     |

We claim:

1. A process for the single-bath dyeing of a fibrous blend of cellulose fibers and synthetic polyamide fibers with a reactive dyestuff and a non-reactive metal complex dyestuff in a continuous or semi-continuous procedure of the pad-dyeing technique which comprises applying to a fibrous blend of cellulose fibers and polyamide fibers an aqueous alkaline padding liquor containing a reactive dyestuff for said cellulose fibers and a non-reactive metal complex dyestuff for said polyamide fibers, padding the fibrous blend thus treated with said padding liquor, and then fixing said reactive dyestuff on said cellulose fibers and said non-reactive

metal complex dyestuff on said polyamide fibers by allowing said fibrous blend to dwell between 2 and 24 hours in moist condition at about room temperature or at slightly elevated temperature.

60 2. A process according to claim 1 wherein said fibrous blend is wound-up and allowed to dwell at about room temperature.

3. A process according to claim 1 wherein said fibrous blend is wound-up and allowed to dwell at a temperature of about 30° to about 60°C.

65 4. A process according to claim 1 wherein said aqueous alkaline padding liquor contains, as a capillary-active mixture, a branched-chain aliphatic carboxylic

acid ester, a partially saponified phosphoric acid ester of an aliphatic alcohol of medium molecular weight, a fatty acid or soap, and a higher oxalkylate of an aliphatic or an aliphatic-aromatic sulfonic acid wetting agent.

5. A process according to claim 1 wherein said aqueous alkaline padding liquor contains an alkali metal salt of m-nitrobenzene sulfonic acid as an auxiliary agent.

6. A process according to claim 1 wherein said aque-

ous alkaline padding liquor contains a polyalkylene glycol of average molecular weight of about 400 to about 800 as an auxiliary agent.

7. A process according to claim 1 wherein said reactive dyestuff has a vinylsulfone group or a group which forms a vinylsulfone group in alkaline medium.

8. A process according to claim 1 wherein said dwell is between 8 and 14 hours.

\* \* \* \* \*

10

15

20

25

30

35

40

45

50

55

60

65